

## UNITED STATES PATENT OFFICE.

ELMER C. PFEIL, OF FOSTORIA, OHIO, ASSIGNOR TO CENTRAL RAILWAY SIGNAL COMPANY, OF PITTSBURGH, PENNSYLVANIA, A CORPORATION OF NEW JERSEY.

## COMPOSITION FOR RAILWAY SIGNAL FUSEES.

No Drawing.

Application filed August 29, 1918. Serial No. 251,911.

To all whom it may concern:

Be it known that I, ELMER C. PFEIL, a citizen of the United States, residing at Fostoria, in the county of Seneca and State of Ohio, have invented certain new and useful Improvements in Compositions for Railway Signal Fusees, of which the following is a specification, reference being had thereto in the accompanying drawing.

10 This invention relates to improvements in compositions for railway signal fusees, which will meet all of the complex requirements imposed upon railway time burning signal fusees by the conditions under which 15 such signals are used, and which will not be subject to spontaneous ignition.

Heretofore, only two types of railway time burning signal fusees have ever been commercially used by the railroads, so far 20 as I am aware, after years of practical experience by me in the manufacture and sale of railway signals, and these two types have become well known to those skilled in this art as

25 First: The "chlorate fusee" and  
Second: The "perchlorate fusee."

The first type, was exclusively commercially manufactured and sold, and exclusively used by the railroads for fully twenty 30 years, before the discovery of the second type of fusee. The first type (chlorate fusee) was subject to spontaneous ignition, and caused much damage to property and life because of that known defect.

35 After the discovery and commercial manufacture of the second type (perchlorate fusee) which overcame the defect of spontaneous ignition, the Bureau for the Safe Transportation of Explosives, by its specification prohibited the transportation of the 40 dangerous chlorate fusee, and since that time the perchlorate fusee has been exclusively manufactured, and exclusively used by railroads. The practical requirements of rail-

45 way signal fusees, may be briefly summarized to be burning in all kinds of weather; burn when submerged in a snow bank or in a puddle of water; burning a predetermined specified time under such conditions; burning with brilliancy and force of flame under said conditions; consuming the tough fiber tube uniformly with the composition which is tightly packed therein to prevent "chimneying"; withstanding 50 the shock of being thrown from a rapidly

running train without breaking and without being extinguished; capable of being readily kindled; capable of free burning at the lowest practical temperature, and at the same time not be subject to spontaneous combustion irrespective of its age.

60 The "perchlorate" fusee is the only fusee known to me that has commercially met the foregoing requirements. In devising a fusee composition, there are conditions to be 65 met beyond the mere action of the chemicals upon each other, as they must collectively act as required when tightly packed in a tough tube, and they must collectively act to consume the tough tube uniformly with 70 the burning of the tightly packed composition. So a railway time burning fusee composition is more than the mere mixing of certain chemicals.

75 For the above reasons, the production of a chemical composition for railway signal fusees which will serve successfully all the requirements imposed upon it, has long been recognized as a very difficult problem. And for these reasons, although many different 80 compositions have been proposed, the only one known to me today which commercially and successfully meets these requirements is the "perchlorate" fusee, and, in fact, it is 85 the only type of railway signal fusee that is today manufactured and used.

The "perchlorate" fusee formula, as used today is perchlorate; sulphur; carbohydrate (in the form of greased sawdust) a strontium nitrate for color, and charcoal.

90 Perchlorate has for some time been difficult to obtain, and is very expensive. Because of the scarcity and expense of perchlorate those skilled in the art have endeavored to either

95 (1) Produce a fusee compound without perchlorate which would meet the requirement, or

(2) Reduce the amount of perchlorate to such an extent that the foregoing troubles 100 would become substantially negligible.

After much thought and experimentation, I have been able to produce a railway time burning signal fusee composition, which will meet all the requirements, entirely without 105 perchlorate, to which preferably so little perchlorate is added as to make the commercial use thereof not objectionable.

My new railway time burning signal fusee composition consists of the following in- 110

2  
gredients, which are compounded preferably in about the quantities given:

|    | Pounds.                 |
|----|-------------------------|
| 5  | Nitrate of potassium 22 |
|    | Sulphur 25              |
|    | Strontium nitrate 130   |
|    | Rosin 4                 |
|    | Red gum 3               |
| 10 | Charcoal 3              |

10 The sulphur is primarily for causing the tough paper tube in which the composition is contained to burn away substantially uniformly with the burning of the composition. 15 Rosin, red gum and charcoal constitute combustibles, which regulate the time of burning of the composition, and the nitrate of potassium is the oxidizing agent which maintains the composition in high winds, rain storms, etc., and even if submerged in a snow bank and irrespective of its position and if submerged in water.

I find that the force of flame of the above composition is somewhat increased, by adding thereto 5 pounds of potassium perchlorate, and reducing the amount of nitrate of potassium to 17 pounds.

All these ingredients are thoroughly mixed and tightly packed in a tough fibre tube.

30 My new fusee composition is found in actual practice to meet all of the herein mentioned complex requirements imposed upon such signals, and it avoids the objectionable use 35 of perchlorate because of the difficulty in obtaining it and the price thereof when obtained.

The "perchlorate" fusee composition requires either a carbohydrate or a hydrocarbon for its successful burning, which is not 40 true of my fusee compound.

The proportions of the ingredients herein given may be varied somewhat without departing from the essentials thereof, but so 45 far I find that the proportions herein given produce the best result.

Fireworks are sometimes confused with railway time burning signal fusees, but they

are recognized by those skilled in the two practical arts, as entirely apart from each other, in that railway signal fusees must meet conditions and requirements which are foreign to fireworks, and the two problems are very different.

Having thus described my invention, what I claim and desire to secure by Letters Patent are—

1. In a railway signal fusee, the combination with a tough fibre tube of a chemical compound packed therein, comprising only 60 nitrate of potassium, sulphur, strontium nitrate, a regulating combustible in about the proportions specified, whereby it is not subject to spontaneous ignition, consuming the tube uniformly with the burning of the composition, burns in high winds, rain snow and is not subject to being extinguished when thrown from a rapidly moving train.

2. In a railway signal fusee, the combination with a tough fibre tube, of a composition 70 packed therein comprising nitrate of potassium, sulphur, strontium nitrate and a time regulating combustible, the parts being in the proportions specified whereby the tube is consumed uniformly with the burning of the compound, the compound burning in the presence of high winds, snow, rain, and not subject to extinguishment when thrown from a rapidly moving train.

3. A time burning railway signal fusee 80 composition, comprising the following ingredients in substantially the following proportions: nitrate of potassium 22 pounds, sulphur 25 pounds, coloring metallic nitrate 130 pounds, and time regulating combustibles 10 pounds, producing a cheap time burning fusee composition burning under the conditions specified and not subject to spontaneous combustion.

In testimony whereof I hereunto affix my signature in the presence of two witnesses

ELMER C. PFEIL.

Witnesses:

JOHN D. SNYDER,  
W. M. WITHERSPOON.